

# UNITED STATES PATENT OFFICE.

ERNST ULRICHS, OF ELBERFELD, GERMANY, ASSIGNOR TO THE FIRM OF WÜLFING, DAHL & CO., ACTIENGESELLSCHAFT, OF BARMEN, GERMANY.

## AZO LAKE AND PROCESS OF MAKING SAME.

No. 910,030.

Specification of Letters Patent.

Patented Jan. 19, 1909.

Application filed September 4, 1907. Serial No. 391,354.

*To all whom it may concern:*

Be it known that I, ERNST ULRICHIS, a subject of the King of Prussia, German Emperor, and resident of Elberfeld, Province of the Rhine, German Empire, have invented 5 new and useful Improvements in the Manufacture of Azo Lakes, of which the following is an exact specification.

Lakes from azo-colors are at present manufactured, as is well known, in such manner that the formation of lakes in the presence or in the absence of substrata or with simultaneous formation of substrata, takes place in accordance with one of the following methods. From azo-dyes without sulfo-group, insoluble lakes are prepared in such manner that the combination of the diazo-compound with the other components, for instance of paranitranilin with beta-naphthol takes place in the presence or absence of fatty acids, colloids etc. When azo-colors with one or more sulfo-groups are used, the lake is prepared in such manner that easily soluble sodium salts, such as for instance orange II B, Ponceau 2 R etc. are dissolved 10 boiling and then precipitated with metal salts. Azo-colors of the above class which are soluble with difficulty even in the form of their sodium salts, such as for instance lithol and lake red, are treated boiling or at 15 an ordinary temperature and while in suspension with a solution of metal salts until the decomposition has taken place. Therefore in the case of azo-colors with sulfo-groups always a double reaction takes place. 20

This invention relates to a process for manufacturing insoluble azo-lakes from azo-dyes with one or more sulfo-groups in which the metal salts are obtained not by double 25 decomposition, but the formation of the dye and of the lake takes place in one operation, which begins direct with metal salts of the sulfo-acids or is carried on in such manner that at the end of the combination, all the sulfo-groups are bound to metals. It is true 30 that previously a process has been described in which the inventor has tried to combine in one operation the formation of an azo-dye and the precipitation of a lake, but in that case there is still the double decomposition. It was thought that the conditions for the reaction must be chosen in such manner as to form first the alkali salt which immediately afterwards enters into reaction with 35 the metal salt. Moreover while in such a

process it is only a question of azo-colors with sulfo-groups in the second component, the process according to this invention can be applied also to azo-colors with sulfo-groups in the first component, or even in both components. The process, has therefore, the following advantages. 40

1. As according to the new process the formation of sodium salt of the azo-dye is done away with, the soda required for forming the sodium salt, is economized, and also the hydrochloric acid required for converting metal carbonates into metal chlorids, moreover the manufacture is reduced by one operation. 45

2. In the prior process hereinbefore referred to common salt is obtained as impurity: (a) during the diazotizing, (b) during the combination, (c) owing to the reaction of the sodium salt of the azo-dye with metal chlorids. According to this process, as the reaction of the sodium salt is completely done away with, the lake is obtained from the beginning in a much purer form. Moreover, the formation of a common salt can be 50 still further avoided by carrying on the diazotizing with hydrochloric acid which is subsequently utilized as a substratum by means of a barium carbonate. The lakes need, therefore, very little washing. 55

3. The lakes are obtained direct with the full depth of their color, they require, therefore, to be ground only for a short time, while lakes prepared from azo-colors soluble with difficulty, such as lithol-red and lake-red, had to be ground for several hours. Therefore in case where the corresponding dye itself or the corresponding substratum, as for instance minium, become duller when subjected to long grinding this process is of 60 a considerable advantage for obtaining clear shades. 65

4. At the double decomposition of sodium salts with metal salts, dye not precipitated is often mechanically carried down. If such a lake is then subsequently ground the soluble salt of sodium of the azo-dye is again rendered free. The lake is then no longer water-proof, which is often noticeable in printing and lithographic ink. Naturally 70 the above drawback is avoided by the process according to this invention. 75

5. According to the process of this application, not only the old shades can be obtained which are produced by the reaction 80

of the sodium salts with metal salts, but quite considerable changes of shade are brought about by tricks or additions during the combination, and therefore lakes can be produced of such fast color as was hitherto absolutely impossible to produce. As such additions oleic acid, palmitic acid, stearic acid, Turkey red oil, glue, gum, albumin, tragacanth, starch, glycerin could be used.

10 6. Dyes with two or more sulfo-groups which hitherto could not be precipitated, or only with great difficulty, as the sodium of their salts could be only partially replaced by other metals, are rendered useful for the 15 lake industry, as of course the binding of all the sulfo-groups to metals can be obtained.

7. It is further possible to produce double lakes which contain two metals in one molecule of dye, by binding for instance the 20 sulfo-groups of one component to barium, and of the other component to calcium. Of course, the process can also be carried out in such way that, after the combination, the sulfo-groups of one component are already 25 bound to a metal, while the sulfo-groups of the second component which are bound to an alkali, are only then treated with solutions of metal salts. Further the operation can be carried on in such manner that 30 in the case of sulfo-acids with several sulfo-groups, the single sulfo-groups can be bound to different metals, for instance, in the case of disulfo-acid, one sulfo-group is bound to barium, and the other to copper.

35 8. In dyes containing naphthol in the second component, soda-lye can be replaced by other solvents, for instance, Turkey red oil, soaps, barium and calcium hydroxid.

9. As combination agents, could be used in 40 the process according to this invention, cheap carbonates and hydroxids such as witherit, chalk, lime etc.

Compared to the old process, the process according to this invention is therefore considerably cheaper, better and simpler.

45 A few examples will explain the same.

(a) *Sulfo-Groups in the First Component.*

50 Example 1. 17.3 kg. of sulfanilic acid, 10 kg. of carbonate of barium are converted boiling into sulfanilate of barium. The solution is mixed with 25 kg. of hydrochloric acid of 19° Bé. cooled to 0° and diazotized 55 with 7 kg. of sodium nitrite in 70 liters of water. After the free hydrochloric acid has been neutralized by the addition of carbonate of barium, the diazo-compound is introduced into a solution of 14.5 kg. naphthol, 4 kg. of acid and 15 kg. of Turkey red oil of 60 50%. After the combination has been converted, 1200 kg. of a paste of hydrate of alumina are added. The lake produced, which can be used as printing and litho-

graphic ink, is considerably more red than 65 when prepared without Turkey red oil.

Example 2. 22.3 kgs. of naphthyl-amin-sulfo-acid 2.8 are dissolved boiling with 5 kg. of chalk, and 25 kg. of hydrochloric acid of 19° Bé. are added. The free sulfo-acid 70 again separated is then diazotized at about 20° with a solution of 7 kg. nitrite. After having neutralized the excess of hydrochloric acid with chalk, the beautiful yellow diazo-compound is introduced into the 75 following mixture. 14.5 kg. beta-naphthol in powder are mixed with water, then milk of lime, prepared from 2.8 kg. of caustic lime, is added, and also 500 kg. of heavy spar are added. After having introduced 80 the diazo-compound, further quantities of milk of lime are added until, after several hours stirring, there is a slightly alkaline reaction. Then the lake becomes of a beautiful cinnabar red which can be used as oil 85 paint, which adheres well to the surface to be painted, and is subjected to further treatment in the usual manner.

(b) *Sulfo-Group in the Second Component.* 90

Example 3. 10.7 kg. toluidin and 25 kg. hydrochloric acid of 19° Bé. are dissolved in water, cooled with ice and diazotized with a solution of 7 kg. of nitrite. After 95 the diazo-compound has been mixed with cold solution of 70 kg. of crystallized Glauber salt, it is introduced into the following mixture:—32.4 kg. of naphthol-sulfo-acid 1.5 are converted into a salt of barium 100 with the equivalent quantity of carbonate of barium. To this is added a solution of 50 kg. of barium chlorid, then 15 kg. of barium carbonate and 300 kg. of orange minium are added. If, after several hours of stirring, there is still a small quantity of diazo-compound, as much milk of lime is added as necessary to cause the last traces of the diazo-compound to combine. The cinnabar imitation thus prepared has at once its full 105 depth of color, so that it need be ground only for a short time.

Example 4. 30.4 kg. of naphthol-di-sulfo-acid 2.3.6. are converted into salt of barium by boiling with 20 kg. of carbonate of 115 barium. To that are added 5 kg. of chalk and 500 kg. of fixed white in paste form. Then there is added the diazo-compound made in the usual way from 12.1 kg. of xylidin, 25 kg. of hydrochloric acid of 19° 120 Bé. and 7 kg. of nitrite. Milk of lime is slowly added until the combination is complete. The lake produced can be used in the form of paste as paint for wall papers.

(c) *Sulfo-Groups in Both Components.*

Example 5. 30.3 kg. of naphthyl-amin-di-

sulfo-acid 2.3.6; and 10 kg. of chalk are dissolved boiling. 25 kg. of hydrochloric acid of 19° Bé. are added, and the whole is diazotized at 20° with the solution of 7 kg. nitrite. 5 The yellow diazo-compound is introduced into the following solution:—30.4 kg. naphthol-di-sulfo-acid 2.3.6 are dissolved boiling with 10 kg. of chalk. To that are added 200 kg. of kaolin and 200 kg. of heavy spar, and 10 then milk of lime is slowly added until the formation of dye stuff is completed.

Example 6. The operation is carried on in the same way as in Example 5, with the difference that 30.4 kg. of naphthol-di-sulfo-15 acid 2.3.6. are converted into salt of barium in the usual manner. The lake produced in which the two-sulfo-groups are combined with barium and two to calcium is considerably more blue than the previous one.

20 Having thus fully described the nature

of my invention, what I desire to secure by Letters Patent of the United States is:—

1. A process of making azo-lakes which consists in forming the dye simultaneously with the precipitation of the lake in the absence of alkali so that the sulfo-groups are all united directly to metallic constituents. 25

2. A process of making azo-lakes which consists in forming the dye simultaneously with the precipitation of the lake in the absence of alkali so that the sulfo-groups are all united directly to metallic constituents, 30 said reaction being carried out in the presence of fatty acids.

In witness whereof I have hereunto set 35 my hand in the presence of two witnesses.

ERNST ULRICHHS.

Witnesses:

WILLIAM MAYNER,  
HENRY HASPER.